

April 20, 1948.

J. A. BRUSSET

2,440,005

FINELY DIVIDED CRYSTALLINE LIMESTONE IN HEAVY FLUID  
FOR FLOAT-AND-SINK CONCENTRATION  
Filed March 19, 1945

Fig. 1.



Fig. 2.



Fig. 3.



Inventor:

Jean Albert Brusset,

By

Pierce & Schefler

his Attorneys

## UNITED STATES PATENT OFFICE

2,440,005

FINELY DIVIDED CRYSTALLINE LIMESTONE  
IN HEAVY FLUID FOR FLOAT-AND-SINK  
CONCENTRATIONJean Albert Brusset, Blairmore, Alberta, Canada,  
assignor to McNally Pittsburg Manufacturing  
Corporation, Pittsburg, Kans.Application March 19, 1945, Serial No. 583,608  
In Canada July 20, 1944

4 Claims. (Cl. 209—173)

1

This invention relates to the art of cleaning coal by a gravity concentration of the float-and-sink type, and is particularly concerned with the provision of an improved suspending medium or "heavy fluid" for use in the said process of separating coal from slate and other refuse.

In such processes, the suspending solid is so selected, and the proportion of solid to suspending liquid (usually water) usually is so adjusted that the resulting "heavy fluid" has a specific gravity varying, according to requirements of each special coal, between 1.30 and about 1.70. There are a great many solids having specific gravities which would be operable were specific gravity the only criterion; however, there exist a number of other criteria which, in effect, greatly narrow the field of operable solids.

Contrary to the prior art proposals, the new flotation medium of the present invention consists essentially of an aqueous suspension of finely divided, hard crystalline limestone rock (specifically metamorphosed limestones of the consistency of marble) of high purity, particularly as regards freedom from quartz, shales and clay, said aqueous suspension being in sufficient concentration to provide a medium of required specific gravity. The limestone, which should have a hardness of 3 or only very slightly less than 3, should be as free as possible from shales and clay, in order to minimize the introduction of ultrafine particles into the medium: it should be as free as possible from quartz, in order to depress abrasion of the equipment in which the medium is handled. I have found that properly subdivided, hard crystalline limestone rock of the purity described, deposits of which occur in the Province of British Columbia, Canada, and elsewhere throughout the Dominion of Canada and the United States of America, makes very stable suspensions in water, and all specific gravities of flotation medium, between 1.30 and 1.70, can readily be provided without undue viscosity of the medium at the higher values. The limestone particles desirably resist disintegration during use and handling of the medium containing them and their aqueous suspension does not tend to become colloidal in character.

I have discovered that for optimum separation

2

of coal from shale, slate and other heavy refuse the hard crystalline limestone rock should be so ground or otherwise subdivided that substantially all of the material is minus 48 mesh, that from about 30 to about 35% thereof is minus 48 plus 100 mesh, that from about 40 to about 50% thereof is minus 100 mesh, and that from about 20 to about 25% is minus 200 mesh. The subdivided limestone rock may contain a few percent of plus 48 mesh particles, say, 5% of minus 40 plus 48 mesh material, without destroying its operability.

The suspension medium of the present invention, consisting of an aqueous suspension of the aforesaid subdivided limestone, possesses a number of advantages over previously proposed media; thus, the solid ingredient, viz., the hard crystalline limestone of desirable purity, is readily and widely available; it is easily reduced to the required mesh, and, in the course of being subdivided, does not tend to yield a large amount of ultrafine particles; in use it does not quickly disintegrate to colloidal particles; it is not abrasive on the machinery; it remains readily in suspension; being desirably free from ultrafine particles, it does not stick to the finished products but rather is easily washed off of them; and it is easily recovered from the wash water by cycloning so that recycling is facilitated.

The special advantages accruing from using 30 a subdivided hard, crystalline limestone rock having the above stated preferred size distribution are: (1) the rate of settling of the resulting water-limestone medium for the specific gravity range 1.30-1.70 is sufficiently low that the medium 35 can easily be kept in suspension; and (2) the viscosity of the medium, at specific gravity 1.30-1.70, with the above preferred size composition is low enough to give a very clean and at the same time rapid separation as between coal and refuse.

The preparation of a "heavy fluid" suspending medium, having a specific gravity anywhere between about 1.30 and about 1.70, from water (or other operable suspending liquid) and the above 45 described suspending solid can be effected by well known technique, to the end that said heavy fluid floats the coal but not the slate or other refuse. The resulting heavy fluid may be used either in

the simple separation of the raw coal into two portions (coal, and heavy refuse); or, it may be used in the somewhat more involved separation of the raw coal into, say, three components, viz., a lightest portion consisting of substantially pure coal, a heaviest portion substantially consisting of heavy refuse, and an intermediate or "middling" portion which may be further dressed, or discarded, or used as such. After the removal of the separated portions of components, these latter may be washed to remove therefrom adhering suspending medium, and the suspending medium may be reformed for reuse in a cyclical repetition of the process. Such cyclical process, and apparatus for use therein, are broadly described in my U. S. Patent No. 2,356,648.

The invention will now be described in further detail with reference to the following specific illustrative example:

The raw material for preparing the suspending solid of the "heavy fluid" was a hard, compact, crystalline limestone rock, of high purity and substantially free from quartz, shales and clay, taken from a deposit at Crowsnest, Province of British Columbia, Canada. The rock had a hardness of 3. The rock analyzed: free  $\text{SiO}_2$ —0.9%;  $\text{CaCO}_3$ —97.5%; oxides of Fe and Al—0.25%;  $\text{MgO}$ —1.25%. This raw material was finely divided, for use in the present process, in the following manner: the rock was crushed first to 2 inches and then to  $\frac{1}{4}$  inch; the  $\frac{1}{4}$  inch material thereupon was ground in a Bradley roller mill until 20% thereof passed a 200-mesh screen. The resulting subdivided limestone had the following particle size distribution:

|                              | Per cent   |
|------------------------------|------------|
| Minus 48 mesh-plus 100 mesh  | about 30.0 |
| Minus 100 mesh-plus 200 mesh | about 50.0 |
| Minus 200 mesh               | 20.0       |
|                              | 100.0      |

It was substantially free from ultrafine (or, colloid-like) particles.

A "heavy fluid" suspending medium for cleaning coal was prepared from this subdivided limestone by agitating 56% by weight thereof with 44% of water, yielding a suspension having a specific gravity of 1.55.

The raw coal was a bituminous coal of 24.10% ash content, mined at the Greenhill Mine of the West Canadian Collieries Limited, Blairmore, Alberta, Canada, and screened over a  $\frac{1}{2}$  inch vibrating screen. The resulting separation was of 3 products, as follows:

|                 | Percentage by Weight | Ash Content Per cent |
|-----------------|----------------------|----------------------|
| Clean Coal..... | 65                   | 12.00                |
| Middlings.....  | 8                    | 21.50                |
| Refuse.....     | 27                   | 54.00                |

The above specific example data are typical of the results being obtained in the large scale, commercial working of the above-described process, at the washery of the above-named mine, in the cleaning of a coal of acknowledgedly bad washing characteristics.

At 1.55 specific gravity, it has an index of 17 on the plus-and-minus 0.10% specific gravity distribution curve (see Bureau of Mines Information Circular 7045, December 1938, entitled "An Explanation of Washability Curves for the Interpretation of Float-and-Sink Data on Coal," by G. D. Coe), which means an extremely difficult separation between coal and refuse—as is acknowledged by all experts in coal-washing. The three figures of the appended drawing constitute a set of curves of washability, including the  $\pm 0.10\%$  curve, as determined by laboratory tests on the 0.5"–5.0" portion of this coal, said curves having been derived from the data set out in the three gravimetric analyses and ash distribution Tables I, II and III immediately following:

I. Re Fig. 1; size range, minus 5 in., plus  $1\frac{1}{8}$  in.

| Specific Gravity |       | Plus-and-minus 0.10 sp. gy. | Actual Products |              | Cumulative   |              |              |              |
|------------------|-------|-----------------------------|-----------------|--------------|--------------|--------------|--------------|--------------|
|                  |       |                             |                 |              | Sinkings     |              | Floatings    |              |
| Sink             | Float |                             | Per cent Wt.    | Per cent Ash | Per cent Wt. | Per cent Ash | Per cent Wt. | Per cent Ash |
| 1.3              | 1.8   | 70.5                        | 9.8             | 6.5          | 90.2         | 28.3         | 9.8          | 6.5          |
| 1.4              | 1.4   | 37.4                        | 43.4            | 12.0         | 46.8         | 43.5         | 53.2         | 11.0         |
| 1.4              | 1.5   | 24.5                        | 13.0            | 23.2         | 33.8         | 50.7         | 66.2         | 13.5         |
| 1.5              | 1.6   | 17.0                        | 5.7             | 31.0         | 28.1         | 54.8         | 71.9         | 14.9         |
| 1.6              | 1.7   | 10.0                        | 5.7             | 31.0         | 28.1         | 54.8         | 71.9         | 14.9         |
| 1.7              | 1.7   | 6.9                         | 1.9             | 35.1         | 26.4         | 56.4         | 73.6         | 15.3         |
|                  |       | 5.0                         | 26.2            | 56.4         | -----        | -----        | 100.0        | 26.0         |

II. Re Fig. 2; size range, minus  $1\frac{1}{8}$  in., plus  $\frac{3}{4}$  in.

| Specific Gravity |       | Plus-and-minus 0.10 sp. gy. | Actual Products |              | Cumulative   |              |              |              |
|------------------|-------|-----------------------------|-----------------|--------------|--------------|--------------|--------------|--------------|
|                  |       |                             |                 |              | Sinkings     |              | Floatings    |              |
| Sink             | Float |                             | Per cent Wt.    | Per cent Ash | Per cent Wt. | Per cent Ash | Per cent Wt. | Per cent Ash |
| 1.3              | 1.3   | 56.1                        | 16.3            | 4.8          | 83.7         | 28.0         | 16.3         | 4.8          |
| 1.4              | 1.4   | 39.7                        | 31.7            | 8.6          | 52.0         | 40.1         | 48.0         | 7.2          |
| 1.4              | 1.5   | 30.1                        | 16.0            | 16.8         | 36.0         | 50.4         | 64.0         | 9.6          |
| 1.5              | 1.6   | 21.9                        | 9.6             | 28.8         | 26.4         | 58.2         | 73.6         | 12.1         |
| 1.6              | 1.6   | 15.5                        | 9.6             | 28.8         | 26.4         | 58.2         | 73.6         | 12.1         |
| 1.6              | 1.6   | 10.5                        | 3.6             | 37.8         | 22.8         | 61.6         | 77.2         | 13.3         |
| 1.7              | 1.7   | 7.2                         | 22.8            | 81.6         | -----        | -----        | 100.0        | 24.3         |

III. Re Fig. 3; size range, minus  $\frac{3}{4}$  in., plus  $\frac{1}{2}$  in.

| Specific Gravity |       | Plus-and-minus 0.10 sp. gy. | Actual Products |              | Cumulative   |              |              |              |
|------------------|-------|-----------------------------|-----------------|--------------|--------------|--------------|--------------|--------------|
|                  |       |                             |                 |              | Sinkings     |              | Floatings    |              |
| Sink             | Float |                             | Per cent Wt.    | Per cent Ash | Per cent Wt. | Per cent Ash | Per cent Wt. | Per cent Ash |
| 1.3              | 1.3   | 64.0                        | 20.0            | 4.7          | 80.0         | 29.9         | 20.0         | 4.7          |
|                  | 1.4   | 53.6                        | 27.4            | 9.0          | 52.6         | 40.8         | 47.4         | 7.2          |
| 1.4              | 1.5   | 41.5                        | 18.4            | 18.5         | 34.2         | 53.0         | 65.8         | 10.3         |
| 1.5              | 1.6   | 30.8                        | 22.0            | 7.9          | 26.3         | 59.6         | 73.7         | 12.5         |
| 1.6              | 1.7   | 13.4                        | 10.5            | 3.6          | 22.7         | 63.6         | 77.3         | 13.6         |
| 1.7              | ----- | 7.6                         | 22.7            | 63.6         | -----        | 100.0        | -----        | 24.9         |

In each of Figs. 1, 2 and 3, curve "I" is the specific gravity curve, curve "II" is the plus-and-minus 0.10% specific gravity distribution curve, curve "III" is the cumulative float ash curve, and curve "IV" is the cumulative sink ash curve.

The industrial plant obtains a better refuse than seems possible under the laboratory tests, because the middlings are separated from the refuse in the large scale plant.

I claim:

1. The method of separating particles of coal from a mixture thereof with particles of heavy refuse, which comprises forming an aqueous suspension of finely divided crystalline limestone substantially free from quartz and from components which tend readily to disintegrate through use and handling into ultra-fine particles, said limestone having a hardness of about 3, practically all of which finely divided limestone is of a degree of fineness to pass a 48 mesh screen, a large fraction thereof being minus 100 mesh and a minor but substantial part thereof, not exceeding about 25% by weight, being minus 200 mesh in particle size, introducing the mixture into a bath of said aqueous suspension of finely divided limestone, adjusting and maintaining the density of the aqueous suspension at such a value that the coal particles float on said bath but the particles of heavy refuse sink therein, and separately removing coal particles and particles of heavy refuse from said bath.

2. A suspending medium for separating coal from a mixture thereof with particles of heavy refuse by the float-and-sink method, said sink-and-float medium being an aqueous suspension, having a specific gravity between 1.30 and about 1.70, of finely divided, hard, crystalline limestone rock having a hardness of about 3, said limestone rock being substantially free from quartz and from components which tend readily to disintegrate through use and handling into ultra-fine particles, practically all of which finely divided limestone is of a degree of fineness to pass a 48 mesh screen, a large fraction thereof being minus 100 mesh and a minor but substantial

part thereof, not exceeding about 25% by weight, being minus 200 mesh in particle size.

3. A suspending medium for separating coal from a mixture thereof with particles of heavy refuse by the float-and-sink method, said sink-and-float medium being an aqueous suspension, having a specific gravity between about 1.30 and about 1.70, of finely divided, hard, crystalline limestone rock having a hardness of about 3, said limestone rock being substantially free from quartz and from components which tend readily to disintegrate through use and handling into ultra-fine particles, at least about 95% of which finely divided limestone is minus 48 mesh, from about 60 to about 75% is minus 100 mesh, and at least about 20% but not more than about 25% is minus 200 mesh in particle size.

4. A suspending medium for separating coal from a mixture thereof with particles of heavy refuse by the float-and-sink method, said sink-and-float medium being an aqueous suspension, having a specific gravity between about 1.30 and about 1.70, of finely divided, hard, crystalline limestone rock substantially free from quartz and from components which tend readily to disintegrate through use and handling into ultra-fine particles, said finely divided limestone having a hardness of about 3 and the approximate size distribution:

|                               | Per cent |
|-------------------------------|----------|
| Through 48 mesh, on 100 mesh  | 30.0     |
| Through 100 mesh, on 200 mesh | 50.0     |
| Through 200 mesh              | 20.0     |

JEAN ALBERT BRUSSET.

## REFERENCES CITED

The following references are of record in the file of this patent:

## UNITED STATES PATENTS

|    | Number    | Name     | Date          |
|----|-----------|----------|---------------|
| 60 | 1,290,516 | Conklin  | Jan. 7, 1919  |
|    | 1,392,399 | Chance   | Oct. 4, 1921  |
|    | 1,524,838 | Muller   | Feb. 3, 1925  |
|    | 2,140,899 | Davidson | Dec. 20, 1938 |
|    | 2,356,648 | Brusset  | Aug. 22, 1944 |